

## UNITED STATES PATENT OFFICE

2,505,048

INCREASING THE TENACITY OF CELLULOSE  
ACETATE YARNS

Thomas Jackson and Frank Brentnall Hill, Spondon, near Derby, England, assignors to Celanese Corporation of America, a corporation of Delaware

No Drawing. Application March 6, 1946, Serial No. 652,484. In Great Britain March 14, 1945

2 Claims. (Cl. 8—132)

1

This invention relates to improvements in the treatment of materials made of organic derivatives of cellulose, and particularly to improvements in the stretching of filaments having a basis of an organic derivative of cellulose.

The stretching of filaments and other materials made of cellulose acetate or other organic derivative of cellulose in wet steam or hot water has been described in a number of prior specifications. For example, U. S. Patent No. 2,142,909 describes a process in which filaments, threads and similar materials of an organic derivative of cellulose are stretched during their passage through an apparatus comprising an end pressure chamber containing compressed air or other inert gas and a stretching chamber containing saturated or wet steam at a temperature above 100° C. In this manner the tenacity of the materials may be increased.

The above process gives excellent results starting from the ordinary commercial filaments of cellulose acetate, namely filaments of the order of 2 to 5 denier. Indeed such results are obtainable with filament deniers considerably higher than the commercial deniers, such as 10 to 15. When filaments having a denier of 2 to 10 or 15 are stretched 10 or 20 times, the resulting filaments have a denier of 0.1 to 1.5. When these filaments are completely saponified to regenerated cellulose, the filament deniers then become of the order of 0.06 to 1 denier. For some purposes strong yarns are required composed of filaments having higher deniers than the extremely fine ones mentioned, for example regenerated cellulose filaments having deniers of the order of 5 to 10. This necessitates starting with filament deniers of 75 to 150. It is frequently found when starting with filaments of such very high denier as 75 to 150, or even lower denier, for instance 25 or 30, that the improvement in the tenacity obtained by stretching is not so great as that obtained when stretching filaments of the ordinary commercial deniers, such as 2 to 5 or 10. This is more particularly the case when the speed at which the filaments are drawn away from the point of stretching is high, for example, 150 to 200 metres per minute at which speed the stretching of lower denier filaments, for example filaments of 5 to 10 denier, can readily be effected to obtain products of good properties.

It has now been found that it is very advantageous if, prior to stretching, filaments made of organic derivatives of cellulose are soaked in water until they are thoroughly wet-out. Most conveniently they are soaked in package form, e. g.

2

in hanks or on bobbins, for a considerable time, for instance for 1, 5, 10 or 20 hours or more. This preliminary soaking enables the filaments to be stretched at higher speeds than can be employed in the absence of the soaking without sacrificing the properties of the products in some measure.

By the term "thoroughly wet out" as applied to the filaments is meant that the filaments are permeated with water and that their water content is a substantial proportion of that which the filaments contain when in equilibrium with water. Preferably the water content is substantially that which the filaments contain when in equilibrium with water. Wetting-out may be assisted by the use of a wetting agent, e. g. an alkyl naphthalene sulphonic acid, a sulphonic acid ester of lauryl, oleyl or other higher aliphatic alcohol or Turkey red oil. Soaking may be carried out at atmospheric temperature or the water may be heated, for example to a temperature of 50 or 70° C.

The value of the soaking is most marked when the stretching is carried out in wet steam, though it is also advantageous if hot water is employed as the stretch-assisting agent.

The stretching conditions which are suitable are similar to those described in U. S. Patent No. 2,142,909. The degree of stretch employed is usually about ten to twenty times, using wet steam or hot water at a temperature between 130 to 145° C. according to the nature of the cellulose derivative, e. g. its viscosity and the kind and proportion of substituent radicles. The higher the viscosity of a cellulose derivative the higher in general is the temperature of the hot water or wet steam which gives the best results, provided that the cellulose derivatives are otherwise comparable, e. g. as regards the degree of substitution and the nature of the substituent radicle. For example, filaments made of an acetone-soluble cellulose acetate of 10 to 20 viscosity give good results when stretched in wet steam at a temperature of 133 to 135° C., whereas if made of one of 80 to 100 viscosity the temperature of the wet steam should be increased to about 143 to 145° C. The viscosities given above are obtained by comparing the rate of flow of a 6% solution of the acetate in acetone at 25° C. with the rate of flow of glycerin under the same conditions. For this purpose the viscosity of glycerin is taken as 100.

Filaments which are to be stretched in accordance with the present invention may be produced by extruding a solution or plastic mass having a basis of cellulose acetate, cellulose propionate, cellulose butyrate, cellulose acetate-butyrate or other organic derivative of cellulose through an ori-

face of such dimensions that filaments of high denier are directly produced, or they may be obtained by coalescing a number of filaments of lower denier, for example as described in British Patent No. 326,462. Thus an acetone solution of cellulose acetate may be spun in an ordinary dry-spinning cell to give a bundle of filaments, each of which has a denier of about 6, and this bundle of filaments on issuing from the cell may be passed over a wick which is impregnated with acetone and from there round a feed roller and over a lubricating wick to a bobbin or other take-up device.

This method gives a coalesced monofilament having a denier, for example, of 120 to 150, according to the number and denier of the filaments in the bundle, which can be stretched by the process of the present invention to give a product having a tenacity of 4 to 5 grams per denier. For instance, three ends of coalesced yarn, each of which has a denier of 150, may be stretched to ten times their original length in wet steam at a temperature of 130 to 145° C. and may then be twisted and wound to give a stretched, high-tenacity yarn of 45 denier.

A further increase in tenacity may be achieved by completely saponifying the stretched filaments to give a product having a basis of regenerated cellulose. A very satisfactory saponifying liquid for this purpose is a 0.5% aqueous solution of sodium hydroxide containing 10% of sodium acetate at a temperature of 60 to 70° C.

The following example is given to illustrate the invention:

*Example*

A monofilament of 150 denier, made as described in British Patent No. 326,462 by coalescing a number of filaments of lower denier having a basis of acetone-soluble cellulose acetate, was soaked in package form in water for sixteen hours. It was then stretched to ten times its original length at an output speed of 150 to 200 M. P. M., while it is passed through wet steam at a temperature of 134.5° C. in an apparatus such as that illustrated in U. S. Patent No. 2,142,909, using water in the end chamber. The stretched filament had a tenacity of about 4.4 grammes per denier, whereas when stretching was carried out without soaking the monofilament in water the tenacity of the stretched filament was only about 3 grammes per denier.

The process of the present invention has been described above in relation to the stretching of

filaments of high denier having a basis of acetone-soluble acetate, since it is for this purpose that it is of greatest importance. It is, however, also applicable to the stretching of filaments made of other organic derivatives of cellulose, e. g. cellulose propionate, cellulose butyrate, cellulose acetate-butyrate and ethyl cellulose.

Having described our invention, what we desire to secure by Letters Patent is:

1. In a process for producing high-tenacity yarns having a basis of an acetone-soluble cellulose acetate and a denier of at least 5 by stretching yarns having a filament-denier of at least 75 by at least ten times their original length in the presence of wet steam at a temperature above 130° C., the improvement which consists in immersing the yarn in package form for at least 16 hours in water at a temperature below 50° C., and subjecting it to the stretching treatment as the next operation.
2. In a process for producing high-tenacity yarns having a basis of an acetone-soluble cellulose acetate and a denier of at least 5 by stretching yarns having a filament-denier of at least 75 by at least ten times their original length in the presence of wet steam at a temperature above 130° C., the output speed of the yarn from the stretching apparatus being at least 150 meters per minute, the improvement which consists in immersing the yarn in package form for at least 16 hours in water at a temperature below 50° C., and subjecting it to the stretching treatment as the next operation.

THOMAS JACKSON,  
FRANK BRENTNALL HILL.

**REFERENCES CITED**

The following references are of record in the file of this patent:

**UNITED STATES PATENTS**

| Number    | Name             | Date          |
|-----------|------------------|---------------|
| 2,051,831 | Dreyfus          | Aug. 25, 1936 |
| 2,070,584 | Dreyfus          | Feb. 16, 1937 |
| 2,142,912 | Moncrieff et al. | Jan. 3, 1939  |
| 2,279,478 | Moncrieff et al. | Apr. 14, 1942 |
| 2,293,825 | Hosfield         | Aug. 25, 1942 |

**FOREIGN PATENTS**

| Number  | Country       | Date          |
|---------|---------------|---------------|
| 332,231 | Great Britain | July 7, 1930  |
| 371,461 | Great Britain | Apr. 20, 1932 |